

# United States Patent [19]

Raw et al.

[11] 3,842,185

[45] Oct. 15, 1974

[54] ALUMINIUM ALLOY CONDUCTOR WIRE

[75] Inventors: Peter Michael Raw, Harrow; Rees Jenkin Llewellyn, Twickenham, both of England

[73] Assignee: British Insulated Callender's Cables, Limited

[22] Filed: Nov. 30, 1973

[21] Appl. No.: 420,592

## [30] Foreign Application Priority Data

Aug. 9, 1973 Great Britain 37870/73

[52] U.S. Cl. 174/23 R, 174/126 R, 174/128

[51] Int. Cl. H01b 1/02

[58] Field of Search 29/193, 180 S; 174/126 CP, 174/126 R, 23, 27, 128, 130

## [56] References Cited

### UNITED STATES PATENTS

|           |         |                |         |
|-----------|---------|----------------|---------|
| 3,261,908 | 7/1966  | Roche et al.   | 174/128 |
| 3,264,404 | 8/1966  | Treby et al.   | 174/130 |
| 3,378,631 | 4/1968  | Edwards        | 174/130 |
| 3,445,586 | 5/1969  | Edwards et al. | 174/130 |
| 3,496,285 | 2/1970  | Slethei        | 174/130 |
| 3,619,480 | 11/1971 | Bauer          | 174/130 |

|           |        |            |         |
|-----------|--------|------------|---------|
| 3,647,939 | 3/1972 | Schoerner  | 174/130 |
| 3,676,578 | 7/1972 | Cahill     | 174/128 |
| 3,795,760 | 3/1974 | Raw et al. | 174/128 |

## OTHER PUBLICATIONS

Standards For Aluminum Mill Products, The Aluminum Assoc., Eighth Ed. 1965, pp. 10, 21, 74.

Metals Handbook, 8th Ed., 1961, Vol. American Soc. of Metals pp. 943-945.

Primary Examiner—A. T. Grimley  
Attorney, Agent, or Firm—Buell, Blenko & Ziesenhein

## [57] ABSTRACT

An aluminium alloy conductor wire consists of between 98.0 and 99.5 weight percent aluminium, between 0.3 and 1.0 (preferably 0.4 to 0.6) weight percent iron, between 0.08 and 1.0 (preferably 0.2 to 0.4) weight percent copper, a maximum of 0.15 (preferably 0.05 to 0.08) weight percent silicon, and trace quantities of conventional impurities. The conductor wire is especially suitable for use as a conductor of a telecommunication cable or as a component element of an overhead electric conductor.

11 Claims, 2 Drawing Figures



PATENTED OCT 15 1974

3,842,185

FIG. 1.



FIG. 2.



## ALUMINIUM ALLOY CONDUCTOR WIRE

This invention relates to elongate members of aluminium alloy suitable for use in forming a conductor, or an element of a multi-element conductor, of an electric cable or an electric insulated wire, all such elongate members hereinafter, for convenience, being included in the generic term "conductor wire".

It is an object of the present invention to provide an improved conductor wire of an aluminium alloy containing iron as the principal alloying constituent which has a higher tensile strength and higher percentage ultimate

drawn, and after annealing each hard-drawn wire at several different temperatures.

TABLE I

|         | Iron Content Wt. % | Copper Content Wt. % | Silicon Content Wt. % |
|---------|--------------------|----------------------|-----------------------|
| Alloy A | 0.51               | trace                | 0.041                 |
| Alloy B | 0.52               | 0.23                 | 0.047                 |
| Alloy C | 0.51               | 0.41                 | 0.043                 |
| Alloy D | 0.50               | 0.61                 | 0.049                 |
| Alloy E | 0.51               | 0.79                 | 0.058                 |

TABLE II

| Alloy | Temperature of Annealing Treatment °C | Electrical Conductivity % IACS | 0.1% Proof Stress MN/m <sup>2</sup> | Tensile Strength MN/m <sup>2</sup> | Elongation % on 250 mm. |
|-------|---------------------------------------|--------------------------------|-------------------------------------|------------------------------------|-------------------------|
| A     | As drawn                              | 61.4                           | 177                                 | 221                                | 1.6                     |
| B     | do.                                   | 60.5                           | 245                                 | 344                                | 1.4                     |
| C     | do.                                   | 59.1                           | 244                                 | 354                                | 1.1                     |
| D     | do.                                   | 58.0                           | 277                                 | 402                                | 1.8                     |
| E     | do.                                   | 57.0                           | 275                                 | 376                                | 1.5                     |
| A     | 200                                   | 62.3                           | 143                                 | 164                                | 0.4                     |
| B     | do.                                   | 60.5                           | 165                                 | 199                                | 0.4                     |
| C     | do.                                   | 60.2                           | 168                                 | 201                                | 0.5                     |
| D     | do.                                   | 60.3                           | 174                                 | 209                                | 0.6                     |
| E     | do.                                   | 59.5                           | 158                                 | 218                                | 0.8                     |
| A     | 250                                   | 62.3                           | 111                                 | 120                                | 1.8                     |
| B     | do.                                   | 61.2                           | 130                                 | 144                                | 8.8                     |
| C     | do.                                   | 60.5                           | 123                                 | 151                                | 10.0                    |
| D     | do.                                   | 60.3                           | 115                                 | 150                                | 9.2                     |
| E     | do.                                   | 60.1                           | 118                                 | 156                                | 12.0                    |
| A     | 275                                   | 62.9                           | 79                                  | 107                                | 26.0                    |
| B     | do.                                   | 61.7                           | 87                                  | 128                                | 18.5                    |
| C     | do.                                   | 61.0                           | 78                                  | 136                                | 17.5                    |
| D     | do.                                   | 60.4                           | 80                                  | 141                                | 16.0                    |
| E     | do.                                   | 59.9                           | 82                                  | 144                                | 16.0                    |
| A     | 300                                   | 62.9                           | 50                                  | 103                                | 31.5                    |
| B     | do.                                   | 61.8                           | 62                                  | 122                                | 22.5                    |
| C     | do.                                   | 60.5                           | 62                                  | 129                                | 19.0                    |
| D     | do.                                   | 59.8                           | 65                                  | 142                                | 16.0                    |
| E     | do.                                   | 59.4                           | 68                                  | 145                                | 16.5                    |
| A     | 350                                   | 63.3                           | 45                                  | 104                                | 27.0                    |
| B     | do.                                   | 61.6                           | 52                                  | 119                                | 22.0                    |
| C     | do.                                   | 60.1                           | 55                                  | 131                                | 19.0                    |
| D     | do.                                   | 59.6                           | 60                                  | 142                                | 16.0                    |
| E     | do.                                   | 58.5                           | 59                                  | 149                                | 16.0                    |

mate elongation than wires of known aluminium alloys which contain similar quantities of iron.

According to the invention our improved conductor wire is composed of an aluminium alloy consisting of between 98.0 and 99.5 weight percent aluminium, between 0.3 and 1.0 weight percent iron; between 0.08 and 1.0 weight percent copper; a maximum of 0.15 weight percent silicon; and trace quantities of conventional impurities.

The copper content of the aluminium alloy preferably lies in the range 0.2 to 0.4 weight percent.

Preferably the iron content lies in the range 0.40 to 0.60 weight percent and the silicon content lies in the range 0.05 to 0.08 weight percent.

A conductor wire in accordance with the present invention has significantly improved tensile strength as compared with that of conductor wires of the same diameter of known aluminium alloys containing similar quantities of iron but only a trace quantity of copper and the improved tensile properties of our improved conductor wire are illustrated by the following results achieved with a conductor wire of a known aluminium alloy (Alloy A) having a diameter of 0.5 mm and with conductor wire in accordance with the present invention (Alloys B, C, D and E) of the same diameter, as

45 The greater improvement in tensile strength of conductor wires of the present invention as compared with that of conductor wires of the known aluminium alloy occurs with the copper content of the aluminium alloy lying in an upper part of the specified range of 0.08 to 1.0 weight percent.

50 Although in some instances conductor wires of the present invention show a slight loss in electrical conductivity as compared with a conductor wire of a known aluminium alloy containing a similar quantity of iron and only a trace quantity of copper, i.e., approximately 0.001 weight percent, the improvement in tensile strength for a given elongation renders our improved conductor wires especially suitable for use in telephone cables and in other cables where a high tensile strength is desirable and a high electrical conductivity is not of primary importance. Moreover, conductor wires in accordance with the present invention, especially those of an aluminium alloy having a copper content in an upper region of the quoted range, display relatively high tensile strength even in the fully annealed condition. In addition, since in some instances conductor wires of the present invention in an unannealed condition, though having a slightly lower electrical conductivity than a conductor wire of a known alu-

minium alloy containing a similar quantity of iron and only a trace quantity of copper, have a tensile strength that is at least 50 percent greater than that of the unannealed conductor wire of the known alloy, unannealed conductor wires of the present invention are especially suitable for use in overhead electric conductors where tensile strength is a primary consideration.

The conductor wire of the present invention may be prepared by any of the known processes for preparing aluminium alloy wire but we prefer to prepare our improved conductor wire by continuously casting a bar of our aluminium alloy and immediately rolling the bar down to rod form, subsequently drawing the rod to the required wire size and finally annealing the wire.

The invention also includes an electric insulated wire comprising a conductor wire as hereinbefore defined provided with at least one covering layer of insulating material, for instance an extruded layer of plastics insulating material, and the invention further includes an electric cable comprising at least one insulated conductor comprising a plurality of conductor wires as hereinbefore defined and, enclosing the insulated conductor or conductors, an outer protective sheath.

The invention further includes a telecommunication cable comprising a multiplicity of insulated conductors, each conductor comprising a conductor wire as hereinbefore defined. The conductors may be insulated with solid or cellular plastics material and the interstices between the insulated conductors and between them and a surrounding water-proof sheath from end to end of the cable length may be filled with a water-impermeable medium of a grease-like nature.

The invention still further includes an overhead electric conductor comprising at least one conductor wire as hereinbefore defined.

The invention will be further illustrated by a description, by way of example, of a telecommunication cable and of an overhead electric conductor each incorporating conductor wires of the present invention with reference to the accompanying drawings, in which:

FIG. 1 is a cross-sectional end view of the telecommunication cable, and

FIG. 2 is a cross-sectional end view of the overhead electric conductor.

The telecommunication cable shown in FIG. 1 comprises twenty-five pairs of insulated conductors each consisting of an aluminium alloy wire 1 of diameter 0.50 mm and an insulating covering 2 of extruded cellular polyethylene of radial thickness 0.014 mm. The aluminium alloy of each wire 1 consists of 99.0 weight percent aluminium 0.59 weight percent iron; 0.32 weight percent copper; 0.07 weight percent silicon and trace quantities of conventional impurities. Wire 1 has an electrical conductivity of 60.7 percent IACS, a 0.1 percent proof stress of 90 MN/m<sup>2</sup>, a tensile strength of 138 MN/m<sup>2</sup> and elongation on 250 mm of 16.9 percent. The assembly of insulated conductors is surrounded by a longitudinally applied, transversely folded polyester tape 4, a longitudinally applied, transversely folded aluminium tape 5 and an extruded polyethylene sheath 6. The interstices between the insulated conductors and between the insulated conductors and the polyester tape 4 are filled with a water-impermeable medium 3 comprising highly refined petroleum jelly.

The overhead electric conductor shown in FIG. 2 is of overall diameter 42.5 mm and comprises a stranded core 11 of seven steel wires each of diameter 4.72 mm

which is surrounded by three stranded layers 12, 13 and 14 of round aluminium alloy wires 15 of diameter 4.72 mm, the direction of lay of the wires of each layer being opposite to that of the wires in the or each adjacent layer. The aluminium alloy of each wire 15 consists of 99.14 weight percent aluminium; 0.5 weight percent iron; 0.3 weight percent copper; 0.06 weight percent silicon and trace quantities of conventional impurities.

10 What we claim as our invention is:

1. A conductor wire composed of an aluminium alloy consisting of between 98.0 and 99.5 weight percent aluminium; between 0.3 and 1.0 weight percent iron; between 0.08 and 1.0 weight percent copper; a maximum of 0.15 weight percent silicon; and trace quantities of conventional impurities.

15 2. A conductor wire as claimed in claim 1, wherein the iron content of the aluminium alloy lies in the range 0.40 to 0.60 weight percent and the silicon content lies in the range 0.05 to 0.08 weight percent.

20 3. A conductor wire composed of an aluminium alloy consisting of between 98.0 and 99.5 weight percent aluminium between 0.3 and 1.0 weight percent iron, between 0.2 and 0.4 weight percent copper; a maximum of 0.15 weight percent silicon and trace quantities of conventional impurities.

25 4. A conductor wire as claimed in claim 3, wherein the iron content of the aluminium alloy lies in the range 0.40 to 0.60 weight percent and the silicon content lies in the range 0.05 to 0.08 weight percent.

30 5. A conductor wire as claimed in claim 1, which has at least one covering layer of insulating material.

35 6. An electric cable comprising at least one conductor comprising a plurality of conductor wires, each conductor wire being composed of an aluminium alloy consisting of between 98.0 and 99.5 weight percent aluminium; between 0.3 and 1.0 weight percent iron; between 0.08 and 1.0 weight percent copper; a maximum of 0.15 weight percent silicon; and trace quantities of conventional impurities.

40 7. A telecommunication cable comprising a multiplicity of insulated conductors, each conductor comprising a wire composed of an aluminium alloy consisting of between 98.0 and 99.5 weight percent aluminium; between 0.3 and 1.0 weight percent iron; between 0.08 and 1.0 weight percent copper; a maximum of 0.15 weight percent silicon; and trace quantities of conventional impurities.

45 8. A telecommunication cable comprising a multiplicity of insulated conductors, each conductor comprising a wire composed of an aluminium alloy consisting of between 98.0 and 99.5 weight percent aluminium; between 0.3 and 1.0 weight percent iron; between 0.08 and 1.0 weight percent copper; a maximum of 0.15 weight percent silicon; and trace quantities of conventional impurities, a water-proof sheath enclosing the insulated conductors and, filling the interstices between these insulated conductors and between them and the cable sheath from end to end of the cable length, a water-impermeable medium of greaselike nature.

50 9. A telecommunication cable as claimed in claim 8, wherein the insulation of each conductor is a plastics material of cellular form.

55 10. An overhead electric conductor comprising at least one stranded layer of wires, wherein at least some of the wires are composed of an aluminium alloy con-

sisting of between 98.0 and 99.5 weight percent aluminium; between 0.3 and 1.0 weight percent iron; between 0.08 and 1.0 weight percent copper; a maximum of 0.15 weight percent silicon; and trace quantities of conventional impurities.

11. An overhead electric conductor comprising a core of metallic elements of high tensile strength and, surrounding the core, at least one stranded layer of

wires each composed of an aluminium alloy consisting of between 98.0 and 99.5 weight percent aluminium; between 0.3 and 1.0 weight percent iron; between 0.08 and 1.0 weight percent copper; a maximum of 0.15 weight percent silicon; and trace quantities of conventional impurities.

\* \* \* \* \*

10

15

20

25

30

35

40

45

50

55

60

65